

# UNITED STATES PATENT OFFICE.

KRISTIAN BENDIXEN, OF COPENHAGEN, DENMARK, ASSIGNOR TO KRISTIAN BENDIXEN AND PETER BENDIXEN, COPARTNERS TRADING UNDER THE FIRM-NAME OF SKIND-FABRIKEN UNICUM, KR. BENDIXEN, P. BENDIXEN AND COMPANY, OF COPENHAGEN, DENMARK.

## PROCESS OF TANNING FISH-SKINS.

Specification of Letters Patent. Patented Feb. 19, 1918.

1,256,974.

No Drawing. Original application filed February 19, 1912, Serial No. 678,473. Divided and this application filed May 7, 1917. Serial No. 167,154.

*To all whom it may concern:*

Be it known that I, KRISTIAN BENDIXEN, subject of the King of Denmark, and residing at Copenhagen, Denmark, have invented 5 a new and Improved Process of Tanning Fish-Skins, of which the following specification is a full disclosure.

This application is a division of my co-pending case No. 678473 filed February 19, 10 1912 and the invention thereof relates to a process for tanning fish skins and the like, which process is particularly suitable for the skins of sharks, porpoises, whales, etc., as it 15 renders it possible to utilize and work up such skins and thereby render them available as leather.

The process is as follows:—

The salted skins or hides are soaked in water until they are rendered quite fresh 20 again. In the case of the skins of the sharks; these are stretched upon frames and dried. After this the spikes or scales are removed with a clean blunt scraper or tanner's knife. The skins are next put into lukewarm water until they are rendered perfectly soft and are then worked over a beam.

They are next plunged into a depilatory and antiseptic solution of 200 liters of water containing either a kilogram of sodium sulfid 30 or a kilogram of white arsenic or raw red arsenic, or half a kilogram of each of these. In this depilatory and antiseptic solution the skins are to remain for about three days, the skins however being turned twice daily. 35 In the case of the skins of whales this treatment in sodium sulfid and arsenic is not absolutely necessary.

After the expiration of the three days, the skins or hides are put into a solution of 200 40 liters of water and a suitable quantity of slaked lime, and in this solution they are also left for about three days, being again turned twice daily.

The skins are next put into a lime-neutralizing solution of 50 liters of water and  $\frac{1}{2}$  liter of hydrochloric acid of the requisite strength and are agitated for about 5 minutes in this solution to dissolve and remove as much as possible of such lime as would 50 otherwise remain in the pores and interfere with the pliability of the ultimate product and are then bated in a bating mill containing 100 liters of water,  $\frac{1}{2}$  bucket of poultry

dung and  $\frac{1}{2}$  kilogram of any preferred chemical bating compound heated to a temperature of about  $18^{\circ}$  C.

After bating the skins are first washed in clean lukewarm water and then in a solution of  $\frac{1}{2}$  liter of hydrochloric acid and 200 liters of water.

The skins are then put into a vat containing a mild dilute solution of conventional tanning material (about  $5^{\circ}$  or  $6^{\circ}$  barkometer) to which liquid a suitable tanning material is added every third day until the 65 skins are thoroughly tanned.

As an alternative, after treatment in the hydrochloric solution, the skins may be placed in a mill with about 4 kilograms of salt and 40 liters of water, and milled for 70 about 10 minutes and then treated with three solutions of graduated strength of chrome tanning material. After this the skins are again milled for about 8 hours and are then left for the night in the mill; milled again 75 on the following day for about 2 hours, and then completely tanned.

The skins after being completely tanned are next put into a mill with pure lukewarm water until they are entirely freed from acid, 80 and are then milled for about 6 hours in a mild relatively dilute solution (about  $5^{\circ}$  or  $6^{\circ}$  barkometer) of sumach extract and water. After this they are colored and then smeared with oil and spread out, dried, damped and smoothed out, polished and bleached. Finally they are rubbed with one part of albumen and 10 parts of water or of 85 skimmed milk to render the skins supple and to prepare them for coloring. They are then 90 glazed and grained.

If the grain does not come out clearly, the skins are placed for about 5 minutes in a solution of one liter of sulfuric acid and 100 liters of water.

As tanning agents the following are given as examples:—

Oakwood or oak-bark, or extract of oak-bark or various other extracts such as quebracho and extracts of gambier.

Having now described the invention, what I claim and desire to secure, is:—

1. A process for tanning fish skins and the like consisting in softening the skins, treating them for about three days in a solution 105 of products produced by chemical action be-

- tween water and arsenic and sodium sulfid, and then treating them for a further period of about three days in a solution of water and slaked lime.
5. 2. A process for tanning fish skins and the like consisting in softening the skins, treating them for about three days in a solution produced by the chemical action between sodium sulfid, water and arsenic, then treating them for a further period of about three days in a solution of water and slaked lime, turning the hides during such treatments, and then agitating the hides in a solution of water and hydrochloric acid.
- 10 3. A process for tanning fish skins and the like consisting in softening the skins, treating them in a solution of products produced by chemical action between water and arsenic and sodium sulfid, then treating them for a further period in a solution of water and slaked lime, turning the hides during such treatment, agitating the hides in a solution of water and hydrochloric acid and then bathing them in a mill containing water and poultry dung and a chemical bathing compound.
- 15 4. A process for tanning fish skins and the like, consisting in softening skins, treating them in a solution of water and arsenic, then treating them for a further period in a solution produced by the chemical action between sodium sulfid, water and slaked lime, turning the hides during such treatments, agitating the hides in a solution of water and hydrochloric acid, bathing them, then removing them into pure lukewarm water, and then into a solution of hydrochloric acid and water.
- 20 5. A process for tanning fish skins and the like consisting in softening the skins, treating them for about three days in a solution of products produced by chemical action between water and arsenic and sodium sulfid, then treating them for a further period in a solution of water and slaked lime, turning the hides during such treatments, agitating the hides in a solution of water and hydrochloric acid, then bathing the hides, then washing them in pure lukewarm water and afterward with a solution of hydrochloric acid and water, then milling them until the skins are fully tanned in a mill containing a suitable solution of salt to which a suitable chrome tanning material is added, then freeing the hides from acid and treating them in a solution of extract of sumach and water.
- 25 6. A process for tanning fish skins and the like consisting in softening the skins, treating them in a solution produced by the chemical action between sodium sulfid, water and arsenic, then depilating them, then bathing them and then milling with a suitable solution of salt to which a suitable chrome tanning material is added; the milling being then continued until the skins are fully tanned, substantially as described.
7. A process for tanning fish skins and the like consisting in softening the skins, treating them with a solution produced by the chemical action between arsenic and sodium sulfid, and ultimately with a suitable solution of salt, to which a suitable chrome tanning material is added.
- 30 8. A process for tanning fish skins and the like consisting in softening the skins, treating them in a solution produced by the chemical action between sodium sulfid, water and arsenic, then treating them for a further period in a solution of water and slaked lime, turning them during such treatments, agitating the hides in a solution of water and hydrochloric acid, then bathing the hides, then washing them in pure lukewarm water and afterward with a solution of hydrochloric acid and water, then milling them until the skins are fully tanned in a mill containing a suitable solution of salt to which a suitable chrome tanning material is added, then freeing the hides from acid and treating them in a solution of extract of sumach and water.
- 35 The foregoing specification signed at Copenhagen, Denmark, this 18th day of April, 1917.

KRISTIAN BENDIXEN.